

# United States Patent

[19]

McGuire et al.

[11] 3,834,533

[45] Sept. 10, 1974

[54] CONCENTRATION OF OXIDE COPPER  
ORES BY FLOTATION SEPARATION

[75] Inventors: Stephen E. McGuire; John C. Stauter; Carl D. Kennedy, all of Ponca City, Okla.

[73] Assignee: Continental Oil Company, Ponca City, Okla.

[22] Filed: Sept. 11, 1972

[21] Appl. No.: 288,200

[52] U.S. Cl. .... 209/166

[51] Int. Cl. .... B03d 1/02

[58] Field of Search..... 209/166, 167

[56] References Cited

UNITED STATES PATENTS

|           |         |                 |           |
|-----------|---------|-----------------|-----------|
| 1,952,907 | 3/1934  | Christmann..... | 209/166   |
| 1,960,526 | 5/1934  | Christmann..... | 209/166   |
| 2,267,205 | 12/1941 | Kyrides.....    | 209/166 X |
| 2,337,118 | 12/1943 | Lontz.....      | 209/166   |
| 2,414,199 | 1/1947  | Gutzeit .....   | 209/166   |
| 2,569,417 | 9/1951  | Jayne .....     | 209/166   |
| 3,425,549 | 2/1969  | Dickson .....   | 209/166   |

FOREIGN PATENTS OR APPLICATIONS

481,623 3/1952 Canada ..... 209/166

1,120,394 12/1961 Germany ..... 209/166

Primary Examiner—Robert Halper  
Attorney, Agent, or Firm—Ronald J. Carlson

[57] ABSTRACT

Oxide copper ores in subdivided form may be concentrated in a flotation separation process by slurring said ores in an aqueous solution of a flotation reagent followed by generating gas bubbles in the slurry to float the oxide copper and recovering the concentrated oxide copper from the surface of the slurry, wherein the floatation reagent is

(I)



II. condensation reaction products of

- A. polybasic amines of the structure  
 $\text{H}_2\text{N}(\text{CH}_2\text{CH}_2\text{NH})_n\text{H}$ , and  
B. organic halides of the structure  $\text{R}^2\text{Y}$

9 Claims, No Drawings

## CONCENTRATION OF OXIDE COPPER ORES BY FLOTATION SEPARATION

This invention relates to the novel use of certain compounds as flotation reagents in producing oxide copper ore concentrates by flotation separation and, in particular, to producing copper concentrates by flotation separation of ores containing copper in oxidized form such as malachite, azurite, cuprite, tenorite and chrysocolla.

Heretofore, flotation separation techniques for concentrating copper ores have been applied to sulfide copper ores due to the availability of suitable flotation reagents, or collectors as they are sometimes called, for these ores such as the xanthates. Generally, in the typical flotation technique the raw ore containing gangue rock along with the copper ore is first pulverized to a finely divided form and slurried with water to form a pulp. The pulp is then charged to a flotation cell along with the flotation reagent and usually a frother (e.g., a hydroxy compound) and a regulating agent to control the pH. With agitation of the slurry the particles of sulfide copper ore are floated to the surface through the action of the flotation reagent, become suspended in the froth and are then continuously removed from the surface of the slurry. The undesired gangue remains behind in the slurry and is discarded in the tailings from the cell.

While the above-described flotation techniques have been in general use in concentrating sulfide copper ores, they have not been utilized to any extent with oxide copper ores. This has been primarily due to the lack of suitable flotation reagents for the direct flotation of the oxide copper ores since these ores are not as readily floated as the sulfide ores. It has been reported in the literature that mercaptobenzothiazole and salts of fatty acids have sometimes been found effective for direct flotation of the oxide ores but, in general, the oxide ores are first subjected to sulfidization to convert them to the sulfide ores and then concentrated by the usual flotation techniques and reagents. This approach obviously has drawbacks and there is considerable interest in the mining industry in developing direct flotation techniques for oxide copper ores.

In accordance with this invention, it has unexpectedly been found that certain compounds are highly effective as flotation reagents concentrating oxide copper ores by flotation separation without the necessity of first subjecting such oxide ores to a sulfidization treatment. These compounds may be described as



wherein

$\text{R}^1$  is hydrogen or a  $-\text{CH}_2\text{COOX}$  radical;  
 $\text{X}$  is hydrogen or an alkali metal atom such as sodium, potassium or lithium; and  
 $\text{R}^2$  is an alkyl radical having six to 18 carbon atoms or a



radical wherein  $\text{R}^3$  is hydrogen or an alkyl radical having one to 14 carbon atoms and  $\text{R}^4$  is an alkylene radical having one to 15 carbon atoms, with the total number of carbon atoms of both  $\text{R}^3$  and  $\text{R}^4$  being in the range of three to 15; and

II. the condensation reaction products of polybasic amines and organic halides.

The compounds of group (I) and their preparation are known in the art as shown in U.S. Pat. Nos.

10 2,804,474 and 3,228,904. In general, they may be prepared by reaction of a primary amine with a halogen-substituted carboxyl-containing compound. Exemplary of the primary amine reactants  $\text{RNH}_2$  are octyl amine, dodecyl amine, octadecyl amine, hexyl amine, ethylbenzyl amine, 2-ethylhexyl amine, tetramethyloctyl amine and butylbenzyl amine. The halogen-substituted carboxyl-containing compounds include chloroacetic acid, iodoacetic acid, bromoacetic acid, sodium bromoacetate, potassium chloroacetate and sodium chloroacetate.

The condensation reaction products of group (II) are derived from polybasic amines of the structure  $\text{H}_2\text{N}(\text{CH}_2\text{CH}_2\text{NH})_n\text{H}$  wherein  $n$  is an integer of 1 to 6 and organic halides of the structure  $\text{R}^2\text{Y}$  wherein  $\text{R}^2$  is as described above in connection with the group (I) compounds and  $\text{Y}$  is a halogen atom such as bromine or chlorine. The preparation of these compounds involves standard condensation reaction techniques and is described in the examples hereinafter. Exemplary of the polybasic amine reactants are ethylene diamine, diethylene triamine, triethylene tetramine, tetraethylene pentamine, pentaethylene hexamine and hexaethylene heptamine. Among the suitable organic halides defined above are included dodecylbenzyl chloride, octyl bromide, tetradecyl bromide, octadecyl chloride, 2-ethylhexyl chloride, hexylbenzyl chloride, hexyl bromide, dodecyl chloride, decylbenzyl chloride, tridecylbenzyl chloride and 2-butyloctyl bromide.

The above-described compounds have been found useful in flotation separation techniques to concentrate oxide copper ores and, particularly, for concentrating low grade ores containing considerable gangue. These low grade ores may contain as little as  $\frac{1}{2}$  percent copper or less, expressed as  $\text{CuO}$ . As previously indicated, flotation separation generally involves subdividing the raw ore, most desirably to an extent wherein each particle is composed as nearly as possible of either the valuable or worthless material only. The subdivided ore is slurried in water, or the water may be added during the subdividing, so as to form a pulp which will normally contain about 10 to 75 percent solids by weight. The flotation reagent is then added to the pulp and gas bubbles are either generated or introduced in the pulp whereby the solid particles containing the oxide copper ore adhere to the gas bubbles and rise to the surface of the pulp for easy removal as a concentrated oxide copper ore. These techniques are well-known in the art and a more complete and detailed discussion may be found in *Flotation* by A. M. Gaudin, Second Edition, 1957, published by McGraw-Hill. It is also desirable to employ a frothing agent and a pH regulating agent in these techniques as explained in that text. A partial list of some common frothers and regulating agents is presented at page 154 of *An Introduction to the Theory of Flotation* by Klassen and Mokrousov, Second Edition, 1963, published by Butterworth and Co. Ltd. (London).

In general, the compounds may be used as the flotation reagent in the flotation separation process in any amount which is suitable to provide the desired flotation of the oxide copper ore. Of course, for economic reasons the amount employed should be the minimum required to achieve the desired results. Generally, amounts in the range of about 0.01 to about 5 pounds per ton of ore will usually be employed with a range of about 0.05 to about 2 pounds per ton of ore being normally preferred. The amount of flotation reagent and the degree of flotation achieved will be dependent, in part, on the pH of the flotation slurry. Thus, in optimizing a particular separation process it is recommended that a series of simple experiments be run using a conventional Hallimond cell, first determining the optimum pH range with a constant flotation reagent concentration and then determining the optimum flotation reagent concentration at a constant optimum pH. These experiments can be conducted as described in the examples to follow.

The following examples will further illustrate the invention:

#### EXAMPLE 1

##### Preparation of Flotation Reagent

A condensation reaction product of group II was prepared in a 100 ml flask equipped with a magnetic stirrer, condenser with drying tube, thermometer and dropping funnel by charging to the flask 0.055 mol KOH and 50 ml absolute ethanol. The flask was heated to 70°C and stirred to dissolve the KOH. 0.05 mol of ethylene diamine was added as one portion and 0.05 mol of dodecylbenzyl chloride was then added dropwise. After addition of the dodecylbenzyl chloride, the reaction mixture was stirred for about 2 hours at 70°C, then cooled to about 25°C and stirred for another hour. The KCl formed in the reaction was removed by filtration and the resulting clear liquid was stripped of solvent to recover the condensation reaction product.

The dodecylbenzyl chloride used in the preparation was a commercially produced material prepared by chloromethylation of a commercially available alkylbenzene derived from propylene tetramer wherein the alkyl has an average of 12 carbons (Conoco AB 515).

the deslimed mineral to a beaker along with 100 ml aqueous solution of the condensation reaction product having a concentration of  $1 \times 10^{-4}$  mol/liter. The pH of the flotation slurry was then adjusted to the desired value using HCl for pH values of 3-4, NaCO<sub>3</sub> for pH values of 5-9 and KOH for pH values of 10-13. The slurry was stirred for a few minutes for preconditioning and then charged to the modified Hallimond cell. Then a total of about 100 cc of air was bubbled through the slurry over a period of 3 minutes during which time the particles of Chrysocolla were floated and recovered through the upper side arm of the cell. At the end of the 3-minute period the test was terminated and the recovered Chrysocolla which was floated was dried and weighed. The remaining Chrysocolla which was not floated was also recovered, dried and weighed. Based on these two determinations the percent recovery (floated Chrysocolla) was calculated. The results of the tests are set forth in the following table:

20

TABLE I

| pH | % Recovery | pH | % Recovery |
|----|------------|----|------------|
| 3  | 17.2       | 9  | 100.0      |
| 4  | 22.3       | 10 | 93.4       |
| 5  | 24.2       | 11 | 75.2       |
| 6  | 47.1       | 12 | 60.4       |
| 7  | 94.5       | 13 | 69.0       |
| 8  | 100.0      | —  | —          |

30

#### EXAMPLE 2

##### Preparation of Flotation Reagent

A condensation reaction product of group II was prepared as described in Example 1 except that 0.05 mol of diethylene triamine was substituted for ethylene diamine.

##### Flotation Separation Tests

Several flotation separation tests were run as described in Example 1 using the above condensation reaction product. In addition to a series of tests at  $1 \times 10^{-4}$  mol/liter concentration a series was run at  $3 \times 10^{-5}$  mol/liter concentration. The results of each series are shown in the following table.

TABLE II

| pH | % Recovery<br>( $1 \times 10^{-4}$ Conc) | % Recovery<br>( $3 \times 10^{-5}$ Conc) | pH | % Recovery<br>( $1 \times 10^{-4}$ Conc) | % Recovery<br>( $3 \times 10^{-5}$ Conc) |
|----|------------------------------------------|------------------------------------------|----|------------------------------------------|------------------------------------------|
| 3  | 48.7                                     | —                                        | 8  | 100.0                                    | 36.6                                     |
| 4  | 45.1                                     | —                                        | 9  | 100.0                                    | 32.4                                     |
| 5  | 77.2                                     | 17.6                                     | 10 | 100.0                                    | 25.5                                     |
| 6  | 90.8                                     | 21.2                                     | 11 | 100.0                                    | —                                        |
| 7  | 100.0                                    | 28.2                                     | 12 | 92.4                                     | —                                        |

##### Flotation Separation Tests

The above-prepared condensation reaction product was evaluated as a flotation reagent in a series of tests involving various pH values using a conventional modified Hallimond tube flotation cell. In each test a flotation slurry was first prepared and then transferred to the cell. The flotation slurry was prepared by desliming a 1 g sample of -48 + 150 (Tyler) mesh Chrysocolla (CuSiO<sub>3</sub> · 2H<sub>2</sub>O) with distilled water and then charging

60

#### EXAMPLE 3

##### Preparation of Flotation Reagent

A condensation reaction product of group II was prepared as described in Example 1 except that 0.05 mol triethylene tetramine was substituted for ethylene diamine.

##### Flotation Separation Tests:

A dual series of flotation separation tests were run as described in Example 2 using the above prepared con-

65

densation reaction product reagent. The results are tabulated in Table III.

TABLE III

| pH | % Recovery<br>( $1 \times 10^{-4}$ Conc) | % Recovery<br>( $3 \times 10^{-5}$ Conc) | pH | % Recovery<br>( $1 \times 10^{-4}$ Conc) | % Recovery<br>( $3 \times 10^{-5}$ Conc) |
|----|------------------------------------------|------------------------------------------|----|------------------------------------------|------------------------------------------|
| 3  | 96.7                                     | 15.1                                     | 8  | 100.0                                    | 39.2                                     |
| 4  | 100.0                                    | 18.9                                     | 9  | 97.1                                     | 30.0                                     |
| 5  | 100.0                                    | 17.7                                     | 10 | 97.1                                     | 30.4                                     |
| 6  | 100.0                                    | 23.0                                     | 11 | 88.9                                     | —                                        |
| 7  | 100.0                                    | 39.5                                     | 12 | 85.5                                     | —                                        |

## EXAMPLE 4

## Preparation of Flotation Reagent

A condensation reaction product of group II was prepared as described in Example 1 except that 0.05 mol tetraethylene pentamine was substituted for ethylene diamine.

## Flotation Separation Tests

A dual series of flotation separation tests were conducted as described in Example 2 using the above condensation reaction product reagent. The results appear in Table IV.

TABLE IV

| pH | % Recovery<br>( $1 \times 10^{-4}$ Conc) | % Recovery<br>( $3 \times 10^{-5}$ Conc) | pH | % Recovery<br>( $1 \times 10^{-4}$ Conc) | % Recovery<br>( $3 \times 10^{-5}$ Conc) |
|----|------------------------------------------|------------------------------------------|----|------------------------------------------|------------------------------------------|
| 3  | 43.1                                     | 10.4                                     | 9  | 100.0                                    | 56.5                                     |
| 4  | 64.1                                     | 11.6                                     | 10 | 100.0                                    | 67.2                                     |
| 5  | 100.0                                    | 12.4                                     | 11 | 100.0                                    | 57.0                                     |
| 6  | 100.0                                    | 12.2                                     | 12 | 100.0                                    | 17.0                                     |
| 7  | 100.0                                    | 12.6                                     | 13 | 44.6                                     | 16.0                                     |
| 8  | 100.0                                    | 27.2                                     | —  | —                                        | —                                        |

## EXAMPLE 5

## Preparation of Flotation Reagent

A condensation reaction product of group II was prepared as described in Example 1 using 0.05 mol dodecylbenzyl chloride, 0.05 mol triethylene tetramine and 0.055 mol KOH. The dodecylbenzyl chloride was derived by alkylating benzene with dodecene-1 in the presence of  $AlCl_3$  and then chloromethylating the product.

## Flotation Separation Tests:

A series of flotation tests using the above prepared reagent were conducted as described in Example 1. The results are shown in Table V.

TABLE V

| pH | % Recovery | pH | % Recovery |
|----|------------|----|------------|
| 3  | 16.5       | 8  | 51.6       |
| 4  | 26.4       | 9  | 59.6       |
| 5  | 17.5       | 10 | 68.9       |
| 6  | 20.7       | 11 | 50.5       |
| 7  | 29.3       | 12 | 26.4       |

## EXAMPLE 6

## Preparation of Flotation Reagent

A composition of group I was prepared in a 250 ml flask equipped with a mechanical stirrer, thermometer and dropping funnel. The flask was charged with about 0.075 mol of tetradecyl amine and 75 ml triethylamine as an acid receptor and solvent. Thereafter, 0.58 mol ethyl bromoacetate was added dropwise while maintaining the flask at temperatures below about 55°C. After complete addition of the acetate the reaction mixture was stirred for about one-half hour while maintaining the temperatures below 55°C. The ester con-

densation reaction product was recovered by filtration and stripping of the triethyl amine solvent and then

treated with aqueous sodium hydroxide to convert the ester to the sodium salt of N-tetradecyliminodiacetic acid. Some small amounts of sodium N-tetradecyliminomonoacetic acid were also present.

## Flotation Separation Tests

A series of flotation separation tests were performed as described in Example 1 using the condensation reaction product prepared above as reagent. However, in this series of tests a constant pH of 9 was employed while varying the concentration of the reagent. The results are tabulated in Table VI

TABLE VI

| Reagent<br>Conc(m/l) | % Recovery | Reagent<br>Conc(m/l) | % Recovery |
|----------------------|------------|----------------------|------------|
| $1 \times 10^{-5}$   | 3.1        | $2 \times 10^{-4}$   | 44.2       |
| $3 \times 10^{-5}$   | 4.0        | $3 \times 10^{-4}$   | 64.0       |
| $5 \times 10^{-5}$   | 4.1        | $5 \times 10^{-4}$   | 76.8       |
| $7 \times 10^{-5}$   | 5.9        | $7 \times 10^{-4}$   | 100.0      |
| $1 \times 10^{-4}$   | 17.6       | —                    | —          |

## EXAMPLE 7

## Preparation of Flotation Reagent

A composition of group I was prepared as described in Example 6 except that hexadecyl amine was substituted for tetradecyl amine. The reagent product was the sodium salt of N-hexyldecyl iminodiacetic acid.

## Flotation Separation Tests

A series of flotation tests were performed as described in Example 1 using the above condensation reaction product as reagent. However, in this series of tests Malachite ( $CuCO_3 \cdot Cu(OH)_2$ ) was used as the oxide copper ore, the pH was a constant 9 and the concentration of the reagent was varied. The results appear in Table VII.

TABLE VII

| Reagent<br>Conc(m/l) | % Recovery | Reagent<br>Conc(m/l) | % Recovery |
|----------------------|------------|----------------------|------------|
| $1 \times 10^{-7}$   | 6.9        | $3 \times 10^{-5}$   | 26.6       |
| $3 \times 10^{-7}$   | 5.3        | $1 \times 10^{-4}$   | 63.4       |
| $1 \times 10^{-6}$   | 4.8        | $2 \times 10^{-4}$   | 73.5       |
| $3 \times 10^{-6}$   | 3.5        | $2.5 \times 10^{-4}$ | 94.3       |
| $1 \times 10^{-5}$   | 13.6       | —                    | —          |

## EXAMPLE 8

## Preparation of Flotation Reagent

A composition of group I was prepared as described in Example 6 except that hexyl amine was substituted for tetradecyl amine. The reagent product was the sodium salt of N-hexyl iminodiacetic acid.

## Flotation Separation Tests

A series of flotation separation tests were performed according to the procedure of Example 1 using the above prepared condensation reaction product as reagent. However, in this series of tests a constant pH of 9 was employed while varying the concentration of reagent. The results are presented in Table VIII.

TABLE VIII

| Reagent Conc(m/l)  | % Recovery | Reagent Conc(m/l)     | % Recovery |
|--------------------|------------|-----------------------|------------|
| $1 \times 10^{-3}$ | 13.2       | $3 \times 10^{-3}$    | 43.5       |
| $3 \times 10^{-3}$ | 12.5       | $1 \times 10^{-2}$    | 45.6       |
| $1 \times 10^{-4}$ | 22.4       | $3 \times 10^{-2}$    | 56.7       |
| $3 \times 10^{-4}$ | 28.5       | $3.82 \times 10^{-2}$ | 57.5       |
| $1 \times 10^{-3}$ | 44.1       | —                     | —          |

## EXAMPLE 9

## Preparation of Flotation Reagent

A composition of group I was prepared as described in Example 6 except that octyl amine was substituted for tetradecyl amine. The reagent product was the sodium salt of N-octyl iminodiacetic acid.

## Flotation Separation Tests

A series of flotation separation tests were performed according to the procedure of Example 1 using the above described condensation reaction product as reagent. However, in this series of tests Malachite ( $\text{CuCO}_3 \cdot \text{Cu}(\text{OH})_2$ ) was used as the oxide copper ore, the pH was a constant 9 and the concentration of reagent was varied. The results appear in Table IX.

TABLE IX

| Reagent Conc(m/l)  | % Recovery | Reagent Conc(m/l)  | % Recovery |
|--------------------|------------|--------------------|------------|
| $3 \times 10^{-5}$ | 21.5       | $3 \times 10^{-6}$ | 3.7        |
| $1 \times 10^{-4}$ | 33.3       | $1 \times 10^{-5}$ | 4.5        |
| $3 \times 10^{-4}$ | 44.6       | $5 \times 10^{-4}$ | 47.4       |
| $1 \times 10^{-3}$ | 74.6       | $7 \times 10^{-4}$ | 55.9       |
| $3 \times 10^{-3}$ | 100.0      | $2 \times 10^{-3}$ | 100.0      |

## EXAMPLE 10

## Preparation of Flotation Reagent

A composition of group I was prepared as described in Example 6 except that decyl amine was substituted for tetradecyl amine and ethylchloroacetate was substituted for ethyl bromacetate. The reagent product was the sodium salt of N-decylinodiacetic acid.

## Flotation Separation Tests

A series of flotation separation tests were performed as described in Example 1 and modified as indicated in Example 9 using the above condensation reaction product as reagent. The results appear in Table X.

TABLE X

| Reagent Conc(m/l)  | % Recovery | Reagent Conc(m/l)  | % Recovery |
|--------------------|------------|--------------------|------------|
| $3 \times 10^{-6}$ | 8.2        | $7 \times 10^{-5}$ | 64.5       |
| $1 \times 10^{-5}$ | 21.6       | $1 \times 10^{-4}$ | 65.8       |
| $3 \times 10^{-5}$ | 46.7       | $2 \times 10^{-4}$ | 72.7       |
| $3 \times 10^{-5}$ | 49.2       | $3 \times 10^{-4}$ | 93.3       |
| $7 \times 10^{-5}$ | 57.8       | $5 \times 10^{-4}$ | 100.0      |

## EXAMPLE 11

## Preparation of Flotation Reagent

A composition of group I was prepared as described in Example 6 except that dodecyl amine was substituted for tetradecyl amine. The reagent product was the sodium salt of N-dodecyliminodiacetic acid.

## Flotation Separation Tests

Several flotation separation tests were run as described in Example 1 using the above condensation reaction product as reagent except that the reagent concentration employed was  $2 \times 10^{-4}$  mol/liter. In addition to a series of tests with Chrysocolla, a series was performed on each of Malachite, Azurite ( $2\text{CuCO}_3 \cdot \text{Cu}(\text{OH})_2$ ), Cuprite ( $\text{Cu}_2\text{O}$ ) and Tenorite ( $\text{CuO}$ ). The results appear in the following table.

Table XI

| Oxide Copper Ore - Chrysocolla ( $\text{CuSiO}_3 \cdot 2\text{H}_2\text{O}$ ) |            |      |            |
|-------------------------------------------------------------------------------|------------|------|------------|
| pH                                                                            | % Recovery | pH   | % Recovery |
| 3.0                                                                           | 22.0       | 7.8  | 48.3       |
| 3.0                                                                           | 24.2       | 7.9  | 57.9       |
| 4.0                                                                           | 26.1       | 8.1  | 65.8       |
| 4.0                                                                           | 32.3       | 9.1  | 100.0      |
| 4.0                                                                           | 40.9       | 9.2  | 100.0      |
| 4.9                                                                           | 71.5       | 9.9  | 100.0      |
| 5.0                                                                           | 100.0      | 10.3 | 89.6       |
| 5.7                                                                           | 80.0       | 11.0 | 79.6       |
| 6.1                                                                           | 98.0       | 11.3 | 36.6       |
| 6.5                                                                           | 39.4       | 12.1 | 51.2       |
| 6.7                                                                           | 39.4       | —    | —          |
| 7.1                                                                           | 55.8       | —    | —          |
| 7.2                                                                           | 59.7       | —    | —          |
| Oxide Copper Ore - Malachite ( $\text{CuCO}_3 \cdot \text{Cu}(\text{OH})_2$ ) |            |      |            |
| pH                                                                            | % Recovery | pH   | % Recovery |
| 4.7                                                                           | 21.7       | 9.2  | 100.0      |
| 5.9                                                                           | 22.0       | 10.1 | 90.5       |
| 7.2                                                                           | 100.0      | 11.1 | 38.5       |
| 8.1                                                                           | 100.0      | 12.1 | 65.1       |
| Oxide Copper Ore - Azurite ( $2\text{CuCO}_3 \cdot \text{Cu}(\text{OH})_2$ )  |            |      |            |
| pH                                                                            | % Recovery | pH   | % Recovery |
| 4.0                                                                           | 12.8       | 9.0  | 89.8       |
| 5.2                                                                           | 19.4       | 10.2 | 88.4       |
| 6.1                                                                           | 72.7       | 11.1 | 61.8       |
| 7.4                                                                           | 85.0       | 12.2 | 38.7       |
| 8.1                                                                           | 100.0      | —    | —          |
| Oxide Copper Ore - Cuprite ( $\text{Cu}_2\text{O}$ )                          |            |      |            |
| pH                                                                            | % Recovery | pH   | % Recovery |
| 3.2                                                                           | 17.4       | 8.0  | 100.0      |
| 4.1                                                                           | 6.1        | 9.0  | 77.4       |
| 5.0                                                                           | 91.7       | 10.0 | 66.6       |
| 5.3                                                                           | 100.0      | 11.0 | 45.3       |
| 5.9                                                                           | 100.0      | 12.1 | 17.7       |
| 6.8                                                                           | 100.0      | —    | —          |
| Oxide Copper Ore - Tenorite ( $\text{CuO}$ )                                  |            |      |            |
| pH                                                                            | % Recovery | pH   | % Recovery |
| 3.0                                                                           | 79.1       | 9.0  | 73.2       |
| 4.0                                                                           | 76.6       | 9.4  | 87.4       |
| 5.0                                                                           | 69.3       | 10.0 | 70.9       |
| 6.1                                                                           | 35.6       | 11.0 | 44.4       |
| 7.2                                                                           | 37.9       | 12.1 | 64.9       |
| 8.1                                                                           | 45.4       | —    | —          |

## EXAMPLE 12

Condensation reaction products formed by reacting dodecyl chloride with triethylene tetramine or tetradecyl bromide with diethylene triamine may typically be used as flotation reagents in the flotation separation of chrysocolla or malachite.

## EXAMPLE 13

N-decylinodiacetic acid, N-octylinodiacetic acid, N-dodecylbenzyliminodiacetic acid and potassium N-octybenzyl-iminodiacetate may typically be used as flotation reagents in the flotation separation of malachite, chrysocolla or azurite.

Thus having described the invention in detail, it will be understood by those skilled in the art that certain variations and modifications may be made without departing from the spirit and scope of the invention as described herein and in the appended claims.

We claim:

1. In a flotation separation process wherein oxide copper ores in subdivided form are concentrated by slurring said ores in an aqueous solution of a flotation reagent followed by generating gas bubbles in the slurry to float the oxide copper and recovering the concentrated oxide copper from the surface of the slurry, the improvement therein which comprises employing a flotation reagent defined by condensation reaction products of

A. polybasic amines selected from the group consisting of ethylene diamine, diethylene triamine, triethylene tetramine, tetraethylene pentamine, pentaethylene hexamine and hexaethylene heptamine; and

B. organic halides of the structure



wherein  $R^2$  is an alkyl radical having six to 18 carbon atoms or a



where  $R^3$  is hydrogen or an alkyl radical having one to 14 carbon atoms and  $R^4$  is an aliphatic hydrocarbon radical having one to 15 carbon atoms, with the total number of carbon atoms of both  $R^3$  and  $R^4$  being in the range of three to 15; and  $Y$  is a halogen atom.

2. A process according to claim 1 wherein the polybasic amines are selected from the group consisting of ethylene diamine, diethylene triamine, triethylene tetramine and tetraethylene pentamine.

3. A process according to claim 1 wherein  $R^2$  is an alkyl radical having six to 18 carbon atoms and  $Y$  is

bromine or chlorine.

4. A process according to claim 1 wherein  $R^2$  is a



radical and  $Y$  is bromine or chlorine.

5. A process according to claim 4 wherein  $R^4$  has one carbon atom.

6. A process according to claim 5 wherein  $R^3$  is an alkyl radical having eight to 14 carbon atoms.

7. A process according to claim 1 wherein about 0.01 to about 5 pounds of flotation reagent per ton of raw ore are employed.

8. In a flotation separation process wherein oxide copper ores in subdivided form are concentrated by slurring said ores in an aqueous solution of a flotation reagent followed by generating gas bubbles in the slurry to float the oxide copper and recovering the concentrated oxide copper from the surface of the slurry, the improvement therein which comprises employing a flotation reagent defined by



wherein  $R^3$  is hydrogen or an alkyl radical having one to 14 carbon atoms and  $R^4$  is an aliphatic hydrocarbon radical having one to 15 carbon atoms, with the total number of carbon atoms of both  $R^3$  and  $R^4$  being in the range of three to 15; and  $X$  is hydrogen or an alkali metal atom.

9. A process according to claim 8 wherein  $R^4$  has one carbon atom.

\* \* \* \* \*